

## UNITED STATES PATENT OFFICE

2,218,586

## MANUFACTURE OF A BASIS FOR FACE POWDER

Matthias Quaedvlieg, Dessau in Anhalt, Germany,  
assignor to Winthrop Chemical Company, Inc.,  
New York, N. Y., a corporation of New York

No Drawing. Application July 26, 1938, Serial  
No. 221,360. In Germany August 26, 1937

3 Claims. (Cl. 167—92)

As a basis for face powder there have been used the zinc, strontium and aluminium salts of fatty acids of high molecular weight, for instance stearic acid and undecanic acid, also the fatty acid salts described in U. S. A. specification No. 1,995,663. They have a good covering power, are strongly adherent and can be well rubbed in. As an extender for these highly valuable materials talc and like earthy materials have long been used; these, however, possess in very low degree the good properties of the aforesaid fatty acid salts, apart from their capacity for being rubbed in.

This invention relates to the manufacture of bases for face powder by treating talc and similar earthy materials with a suitable fatty acid salt in molten or dissolved state. It has been found that in this manner the outstanding properties of the aforesaid fatty acid salts may be imparted to talc, kaolin, china clay or the like when the zinc, strontium and magnesium salts of higher fatty acids are used. When an aqueous solution is used, the talc, for example, is suspended in the aqueous alkali soap solution and the insoluble metal salt is precipitated on the talc by adding a soluble metal salt, for instance zinc chloride, magnesium sulfate or the like. However, a better basis for face powder is obtained by treating talc with zinc stearate or strontium undecanate in a suitable organic solvent, for instance, carbon tetrachloride, xylene, chlorobenzene or the like, if desired at a raised temperature. Talc thus treated has an improved covering power, a remarkable adherence and far excels a mechanically made mixture of talc with zinc stearate for instance.

The following examples illustrate the invention:

Example 1.—Into a solution of 20 parts of zinc stearate in 100 parts by weight of xylene are introduced at 120° C. 100 parts of talc, and the whole is allowed to cool while stirring, then filtered and the solid matter dried.

For making a high class powder there are mixed:

|                       | Parts |
|-----------------------|-------|
| Talc treated as above | 70    |
| Titanium dioxide      | 3     |
| Zinc oxide            | 20    |
| Calcium carbonate     | 2     |
| Magnesium carbonate   | 5     |

Example 2.—100 parts of talc are thoroughly stirred into a solution of 20 parts of sodium undecanate and 0.5 part of a preparation which is a condensation product of hydroxy-alkyl amine with a higher organic acid made as described in Canadian Patent No. 313,993 which corresponds with U. S. A. application Serial No. 340,015, filed February 14, 1929, by Ulrich and Nuesslein.

There is then run in gradually at 90° C. a solution of 6.6 parts of zinc chloride in 150 parts of water, the whole is stirred for a short time, filtered and the solid matter washed and dried.

In the foregoing examples use is made of zinc stearate and zinc undecanate. In the same manner the corresponding strontium or aluminium salts of the said acids or the zinc, strontium or aluminium salts of any fatty acid having at least 10 carbon atoms in its molecule, may be used.

What I claim is:

1. The process for improving the covering power of talc powder when used as a basis for face powder which comprises treating the talc with a fatty acid metal salt of the group consisting of zinc-, strontium-, and aluminium salts of fatty acids containing at least 10 carbon atoms said fatty acid metal salt being in the liquid phase.

2. The process for improving the covering power of talc powder when used as a basis for face powder which comprises treating the talc powder with a solution of a fatty acid metal salt of the group consisting of zinc-, strontium-, and aluminium salts of fatty acids containing at least 10 carbon atoms, and evaporating the solvent.

3. The process for improving the covering power of talc powder when used as a basis for face powder which comprises treating the talc powder with a melt of a fatty acid metal salt of the group consisting of zinc-, strontium-, and aluminium salts of fatty acids containing at least 10 carbon atoms.

MATTHIAS QUAEDVLIEG.